

May 4, 1965

R. B. COX

3,181,937

ROCKET HYDROFUEL CONTAINER WITH CHEMICAL HEATING DEVICE

Filed Dec. 14, 1954



Fig 1



Fig 2

INVENTOR.  
ROBERT B. COX

BY  
*J. Gordon Angus*  
ATTORNEY

1

3,181,937

ROCKET HYDROFUEL CONTAINER WITH  
CHEMICAL HEATING DEVICERobert B. Cox, Pomona, Calif., assignor to Aerojet-  
General Corporation, Azusa, Calif., a corporation of  
OhioFiled Dec. 14, 1954, Ser. No. 475,053  
2 Claims. (Cl. 44-2)

This invention relates to rocket motors and more particularly to such motors utilizing molten metallic fuels. An object of this invention is to provide a means of readying jet motors utilizing solid metallic fuels for operation in a relatively short time.

It has been proposed to employ metallic hydrofuels such as lithium, potassium, calcium, etc. and alloys of such metals as propellants for such rocket motors. These substances are referred to as hydrofuels because of their spontaneous reaction with water to produce gases useful for propulsion. Such metallic hydrofuels are solids at ordinary temperatures; hence in order to render them useful as rocket hydrofuels they must be heated to the liquid state prior to operation. Thus, the fuel chambers of such rocket engines, as they have been used or proposed up to the present time, have required elaborate arrangements of electrical heating coils or other similar devices which require long periods of time to complete the melting. For example, the melting of the hydrofuel in a typical tank of about 80 lbs. capacity has hitherto required about two hours.

The invention is carried out by positioning a heating tube in the hydrofuel tank in such a manner as to melt the hydrofuel when the heating tube is operated.

A feature is the provision of a non-gaseous heating composition which upon combustion emits a relatively large quantity of heat to effect rapid melting of the hydrofuel.

The foregoing and other features of the invention will be better understood from the following detailed description and the accompanying drawing of which:

FIG. 1 is a cross-section view taken at line 1-1 of FIG. 2 of a hydrofuel storage tank containing a heating tube in accordance with this invention; and

FIG. 2 shows a cross-section view taken at line 2-2 of FIG. 1.

Referring to the drawing, there is shown a storage tank 16 of a generally cylindrical shape containing a centrally located cylindrical heating tube 12. Although the cylindrical shape for tanks will ordinarily be preferred, it should be understood that some other shape such as a square cross-section could be used. The heating tube 12 contains a charge 13 of a substance which can be burned or reacted to produce heat and the tank 16 can be filled almost to the top with a solid hydrofuel 17 such as lithium or any of the other hydrofuels mentioned above, cast in the annular space around the heating tube 12.

The tank 16 is closed by top 22 and bottom 23 so that when the hydrofuel is in liquid condition, gas pressure can be applied at the inlet 18 to force the liquid out the outlet 19.

Alternatively, propellant outlet 19 may be positioned at or near the top of the tank to permit the pumping of propellant as soon as melting begins.

A small amount of space is left empty inside fuel tank 16 to provide space for thermal expansion of the hydrofuel.

2

The heating tube 12 is closed at the bottom and the top opening is closed by a cap 21 through which there is passed a cable 20 leading to an igniting squib 24 related to the heating composition 13.

The heating composition used in the heating tube should be one which does not produce gas during its reaction; otherwise some provision would have to be made for releasing the gas which may not always be convenient or desirable when the tank is used in a device under water.

Because of weight and volume limitations in torpedoes, rockets, and other guided missiles it is necessary that the heating unit of this invention occupy only a minimum amount of space and be capable of releasing large quantities of heat per unit volume. These requirements preclude the use of common commercially available heating compositions such as thermite and others used for such purposes as soldering, etc. because of their relatively low heat release per unit weight. At the same time, it is essential that the amount of heat liberated is not so high as to result in damage to the heating tube itself.

I have found that an excellent composition for use as the heat generating element is provided by a mixture of finely divided aluminum and copper oxide. These substances react according to the following equation:



This is equivalent to 1.0 kilocalorie per gram or 5.1 kilocalories per cubic centimeter.

Other mixtures such as aluminum and lithium or potassium perchlorate, for example, will yield more energy, but unfortunately, it has been found impossible to contain this reaction in a sealed metal tube without the use of special materials in the tube construction. The reaction of a stoichiometric mixture of aluminum and copper oxide is also difficult to contain without the use of costly high melting metal containers, however, I have found that the reaction rate of aluminum and copper oxide can be slowed sufficiently by the incorporation of inert materials such as clay to permit its use in a tube composed of ordinary steel.

The admixture of such materials, however, may in some cases produce difficulties in the burning rate characteristics of the grain, in that burning may be irregular or incomplete due to the presence of such inert materials. I have found that the inclusion of small amounts of other oxidizing materials such as thermite and potassium perchlorate as well as oxidizing agents of comparable strength will correct this defect to provide a grain which will burn in a uniform fashion and emit heat within usable limits.

I have found that a uniform mixture of from 65 to 36% by weight of aluminum and copper oxide in stoichiometric proportions, from 25 to 60% by weight of thermite, and from 4 to 10% by weight of clay, provides a heating composition having the thermal and uniform burning characteristics required for use as the heating composition of this invention. In addition, I have found a second formulation also useful as the heating composition of this invention which comprises from 70 to 92% by weight of aluminum and copper oxide in stoichiometric proportions, from 3 to 15% by weight of aluminum and potassium perchlorate in stoichiometric proportions, and from 5 to 15% by weight of clay.

The following examples are provided to more clearly illustrate the heating compositions useful in the practice of this invention.

## Example I

| Ingredients:            | Percent by wt. |
|-------------------------|----------------|
| Al-CuO (stoichiometric) | 56.1           |
| Thermite                | 37.4           |
| Clay                    | 6.5            |
|                         | 100.0          |

## Example II

| Ingredients:                          | Percent by wt. |
|---------------------------------------|----------------|
| Al-CuO (stoichiometric)               | 83.3           |
| Al-KClO <sub>4</sub> (stoichiometric) | 4.4            |
| Clay                                  | 12.3           |
|                                       | 100.0          |

For use in the heating tube, the foregoing heating substances are powdered, dried, and mixed thoroughly, after which they can be pressed in sections in a suitable tube, such as a steel tube, at pressures in the range of about 40,000 to 80,000 pounds per square inch until a solid grain is obtained. A preferred compacting pressure is about 67,000 pounds per square inch. The high degree of compression not only increases the density of the grain, but also tends to reduce the burning rate which is highly advantageous in the case of a high energy burning mixture which has the tendency to melt the heating tube.

Since great heat is developed at the heating tube 12, this tube itself should be composed of a heat-resistant metal, such as steel. The tube material should have high thermal conductivity and ability to withstand the extremely high temperature developed by the combustion of the high-energy heating grains 13.

In operation the reaction or burning of the heating composition will be initiated by electrical ignition of the squib 24. The heating composition 13 will then commence burning at the end adjacent to the squib, and the entire exposed surface area will react. This reaction will progress down the length of the cylindrical grain of the heating composition. Immediately upon ignition, the hydrofuel 17 in tank 16 will commence to melt in the region adjacent the burning heating composition, this being the region immediately surrounding the cylinder 12. Thus, even though all of the hydrofuel in the tank 16 has not yet melted, there will nevertheless be enough of it in molten condition between the inlet and outlet conduits 18 and 19 so that the liquid hydrofuel propellant is immediately available for use. This will permit substantially instantaneous use of the rocket engine with which it is associated. The flow of the propellant will, of course, be initiated by applying pressure at conduit 18 to force the liquid out the outlet 19 into the rocket motor for use in a well known manner.

The heating compositions of this invention burn at a rate of approximately 0.12 in./sec., hence an entire 80-

pound tank of hydrofuel, such as lithium, can be melted in as little as three minutes.

In order to eliminate the possibility of contamination of the fuel by small particles of the heating composition such as those which might result from failure of the wall of the heating tube, a small wire mesh screen may be interposed at propellant outlet 19 to separate such particles from the fuel.

To facilitate the flow of the molten hydrofuel even before it is completely molten, the outlet 18 can conveniently be carried into the interior of the tank 16 into proximity with tube 12.

The heating tubes of this invention may be used either individually or in groups of two or more when it is desired to melt larger volumes or higher melting metals.

I have found that each heating tube will melt approximately 15 times its own volume of hydrofuels such as lithium and lithium alloys.

## I claim:

- 20 1. A fuel unit for rockets which comprises a container substantially filled with normally solid metal rocket hydrofuel, an inlet and an outlet in said container, a heating tube within said container, a solid self-sustaining heating composition within said container, means for igniting said heating composition and pressurization means communicable with said inlet for pumping said hydrofuel out of said container after it has been converted to molten state by combustion of said self-sustaining heating composition.
- 25 2. A fuel unit for a normally solid metallic rocket propellant fuel which comprises a container for said fuel, an inlet and an outlet in said container, a heating tube within the said container, said heating tube containing a solid self-sustaining heating composition and means for igniting said heating composition, said composition comprising a uniform mixture and stoichiometric proportions of clay, copper oxide, aluminum, and an oxidizer selected from the group consisting of potassium perchlorate and ferric oxide.

## References Cited by the Examiner

## UNITED STATES PATENTS

|           |       |                     |
|-----------|-------|---------------------|
| 1,167,944 | 1/16  | Shuman.             |
| 1,838,357 | 12/31 | Bottrill.           |
| 2,016,407 | 10/35 | Wentzel.            |
| 2,020,101 | 11/35 | Brown ----- 266—39  |
| 2,040,407 | 5/36  | Reed ----- 44—3     |
| 2,152,446 | 3/39  | Temple ----- 266—39 |
| 2,352,951 | 7/44  | Geria ----- 44—3 X  |
| 2,680,063 | 6/54  | Shapiro ----- 44—3  |

CARL D. QUARFORTH, Primary Examiner.

ROGER L. CAMPBELL, WILLIAM G. WILES, REUBEN EPSTEIN, Examiners.